

E. GUICHARD.

PROCESS FOR COVERING WITH A PROTECTIVE PLASTIC COATING FLATTENED STRIPS  
AND PRODUCT THEREOF.

APPLICATION FILED SEPT. 9, 1914.

1,230,151.

Patented June 19, 1917.



WITNESSES

Dr. S. Leibman

Bloffe

INVENTOR  
Edgar Guichard  
BY Marvin Co

ATTORNEYS

# UNITED STATES PATENT OFFICE.

EDGAR GUICHARD, OF ETAMPES, FRANCE.

## PROCESS FOR COVERING WITH A PROTECTIVE PLASTIC COATING FLATTENED STRIPS AND PRODUCT THEREOF.

1,280,151.

Specification of Letters Patent. Patented June 19, 1917.

Application filed September 9, 1914. Serial No. 860,854.

To all whom it may concern:

Be it known that I, EDGAR GUICHARD, a citizen of the French Republic, and residing in Etampes, Seine-et-Oise, France, Moulin 5 de la Pirouette, engineer, have invented certain new and useful Improvements in and Relating to Process for Covering with a Protective Plastic Coating Flattened Strips and Product Thereof, of which the following 10 is a complete specification.

My invention relates to a process for covering flattened strips with plastic material so that the strip in cross section has a covering increasing gradually from the center 15 toward the edges. Hitherto flattened strips have been covered with plastic material so as to have in cross section of the strip a uniform thickness of coating. When a strip uniformly coated is dried the coating there- 20 of contracts, reducing the thickness at the edges. With my process of covering, when the coating on the strips is dry, the contraction of the coating will spread the covering uniformly and the thickness thereof will be 25 the same over the whole cross section of the strip, or, better still, a greater thickness of coating will remain at the edges of the strip so as to more effectively protect the said edges.

30 The accompanying drawings illustrate by way of example a form of machine for carrying the process into effect, this machine being more particularly suitable for covering corset steels with celluloid.

35 Figure 1 is a vertical section of the machine; and

Fig. 2 is an end view on the draw plate from the interior.

The machine shown comprises a hopper *a*, 40 of any suitable form, for the solution of celluloid, which is preferably in a pasty state, that is to say, it will contain only a comparatively small proportion of solvent. The hopper is supported by an operating chamber *b*, with which it communicates. On 45 one side of the chamber is a guide *c* for introducing the steels to be covered. Alining with the guide *c* is another guide *d* positioned within the chamber *b* and leading to a draw plate *z*. The draw plate has an 50 opening *j* the size of which can be varied by the elements *e* and *f* provided at the inner side of the draw-plate and adapted to be regulated by means of the screws *g* and *h* 55 respectively. The ends of these elements

are rounded, as shown in Fig. 2, and with the rounded ends *i* of the groove *j* the same coöperate, so that the space between the steel and the sides of the openings in the draw-plate has a greater width at the edges of the 60 steel than at the center of its faces. At the exit from the draw plate there is arranged a drying bench *k* to receive the coated steels issuing from the draw plate.

The covering of the steels is accomplished 65 as follows: The steels, cut to the required length, are introduced by the guide *c* into the steeping chamber *b* wherefrom they are directed by the internal guide *d* in which the steel moves with a certain amount of 70 play to the draw-plate *z*. In the interior of the steeping chamber, and mainly in the hollow space between the rear end of the guide *d* and the draw-plate, the celluloid in solution submerges the steel, and when issuing from the draw-plate it bears a coating 75 of pasty celluloid, the section of the coated steel being exactly of the form of the opening in the draw-plate formed by the rounded edges *i* of the opening and the rounded ends 80 of the elements *e* and *f*. After the steel is withdrawn from the draw-plate it is dried in any suitable manner, either by passing it into a stove heated by steam, hot air, or otherwise, or by passing an electric current 85 through it to raise its temperature. During such drying the celluloid contracts in a known manner. This contraction always takes place from the edges toward the center of the face of the steel with the result 90 that the steel is coated with great regularity over its entire surface but to a greater extent on its edges, which, as is well known, wear out sooner than the face.

It is self-evident that the machine may be 95 utilized for covering continuous strips, which may be carried, by way of example, on a revolving bobbin placed in front of the guide *c* and rolled on to a drum placed on the right side of the bench *k*.

100 From the above description it will be seen that by means of my process steels may be coated or covered with a plastic material so that the coating formed is of a greater thickness at the edges than in the middle of the strip, and, consequently, when such a coated strip is dried the contraction of the plastic material will tend to reduce the thickness at its edges, thus bringing the coating to a substantially uniform thickness over the entire 105 110

strip and, more probable still, leaving a greater thickness at the edges of the strip, which, as previously described, is still more beneficial than the formation of a uniform 5 coating.

I claim:

1. A process for covering flattened strips consisting in coating the strips with material by a single operation so that the thickness of 10 the covering at the edges is greater than in the middle.

2. A process for covering flattened strips consisting in coating the strips with plastic material by a single operation so that the 15 thickness of the covering decreases uniformly from the longitudinal edges toward the middle of the strip.

3. A process for covering flattened strips which consists in covering the strips with plastic material, scraping off the excess of material from the strip in such a way that a larger quantity of the covering substance 20 will remain on the edges of the strip than on the face thereof and the covering formed

will greatly increase from the middle to the 25 edges of the strip.

4. A process for coating flattened strips which consists in covering the strips with plastic material, then scraping off the excess of plastic material to form a coating on the 30 strip, the thickness of which increases gradually from the middle to the edges of the strip, then drying the strip, the coating at the edges being of such a thickness that under contraction its thickness will not become 35 less than the thickness of the coating in the middle of the strip.

5. A flattened strip having a seamless, incasing coating, the cross section of which coating gradually increases from the middle 40 to the edges thereof.

In testimony whereof I have hereunto set my hand at Paris (France), this twenty-first day of August, 1914.

EDGAR GUICHARD.

In the presence of two witnesses:

CHARLES PIERRE REBOUTEL,  
JEAN LALAURET.